

## UNITED STATES PATENT OFFICE.

HENRY E. VAN DERHOEF AND JACKSON B. WELLS, OF ROCHESTER, NEW YORK, AS-SIGNORS TO EASTMAN KODAK COMPANY, OF ROCHESTER, NEW YORK, A CORPORATION OF NEW YORK.

## PROCESS OF TREATING CELLULOSIC FILMS.

No Drawing.

Application filed January 12, 1924. Serial No. 685,906.

*To all whom it may concern:*

Be it known that we, HENRY E. VAN DERHOEF and JACKSON B. WELLS, citizens of the United States of America, residing at Rochester, in the county of Monroe and State of New York, have invented certain new and useful Improvements in Processes of Treating Cellulosic Films, of which the following is a full, clear, and exact specification.

10 This application is a continuation in part of our application, Serial No. 592,843, filed Oct. 6, 1922, for Process of removing dye from tinted cellulosic film.

15 This invention relates to a process of treating cellulosic films, which is capable of removing dye from tinted or colored films and is likewise capable of lessening the curling tendency of cellulosic films. One object of the invention is to provide a relatively inexpensive and easily controlled process for wholly or partially removing dye from tinted cellulosic films and for lessening the curling tendency of cellulosic films. Another object is to provide a process of this character 20 in which the necessary steps do not impair or substantially dissolve the film. Other objects will hereinafter appear.

25 Our invention is especially applicable to the treatment of cellulosic bases or supports for photographic film. It will, therefore, be described in connection with such film by way of example.

As is well known to those skilled in the art, the cellulosic bases or supports for photographic film are substantially impermeable to water and to photographic aqueous solutions, such as fixing baths and the like. For some purposes, such, for instance, as the production of motion picture positive films, the 30 cellulosic support is frequently dyed,—that is, it at least includes a colored or dyed layer. The latter is usually, but not necessarily, on the rear side of the support, such side being defined as that which is opposite to the face 35 which bears the light-sensitive or photographic emulsion. Sometimes during the process of manufacture this colored layer becomes too deep in tint. It is then necessary to reduce the color without substantially dissolving or in any way impairing the base or support. Furthermore this reduction in color must be under sufficient control, so that it can be stopped at the desired point.

After the photographic films have passed through the photographic baths and been 55 dried, a curling tendency manifests itself. Where the rear face of the support is free or uncovered, this tendency may reach an undesirable degree. Of course, films which are coated on the back with a layer, such as gelatine, have very little curling propensity, but in certain types of films, for instance motion picture films, a gelatine backing is not in general use, because it interferes with the 60 drying of the films on the conventional racks. 65 While the curling tendency in motion picture film, particularly the most widely used nitrocellulose ones, may not manifest itself to a harmful extent in a great many cases, nevertheless, when the film is subjected, as 70 it sometimes is, to especially severe conditions, the curling becomes bothersome. It is, therefore, desirable to provide a way for lessening the curling tendency without impairing the film support or substantially 75 dissolving it.

We have discovered a process which solves both the dye-removal problem and the curl-lessening problem. In other words, the steps constituting our process have the inherent 80 property of either removing dye or lessening curling, or doing both of these things simultaneously, according to whether the film to be treated contains dye or not.

In carrying out our process we treat the 85 support, preferably only the rear face thereof, with a solvent of the cellulosic material out of which the base is formed. This treatment is so restricted that there is merely a temporary softening and penetrating action on the support, but the latter is not substantially dissolved, and after drying preserves practically its former appearance. The restriction of the solvent action, so that it does not impair the support, may 90 be effected by controlling the time during which the solvent contacts with the film, by selecting solvents having the desired degree of solvent-power, by regulating the amount of solvent applied per unit area of film 95 surface, by mixing a solvent with a non-solvent, etc. The last named expedient has been found to be especially practicable, and we shall, therefore, describe it by way of 100 illustration.

The cellulosic material most commonly

employed for film supports is nitrocellulose mixed, of course, with the usual modifying substances. The pyroxylin base thus employed, when dyed, has coloring matter 5 mixed throughout the base or in a layer incorporated with the latter. Usually a relatively thin nitrocellulose layer bearing the coloring material forms the rear part or face of the base.

10 If the tint or color is found to be too deep in this rear layer, the film or support may be brought into contact with a bath composed of a solvent such as acetone, preferably toned down with a non-solvent, such 15 as water, say for instance 70 parts of the former to 30 parts of the latter by weight. While the whole support prior to coating with the photographically sensitive layer might be simply immersed in the bath, we 20 prefer, however, to merely bring the rear face of it in contact with the treating bath. Differently stated, the same result is effected if the bath be applied to the rear face of the support. Rollers, wicks, jets, or any 25 other well known expedients in the art may be employed to effect this application of the liquid. The action of the bath is under very accurate control by regulating the time that the film contacts with a bath of given temperature and strength. Room temperatures are ordinarily sufficient and preferred, although a slight heating is permissible if considered desirable for accelerating the 30 action. The action is also facilitated if the liquid is kept in motion while it contacts with the rear face. Any of the well known machines in this art may be used for this purpose. While the rear face of the support may be treated after the photographic 35 coating has been applied to it, nevertheless, we prefer to act upon the substantially cured support or base before it is made up into the finished photographic film. Acetone is a solvent of dyes commonly used.

40 If the film had any original tendency to curl, this treatment greatly lessens it, so that it withstands subsequent photographic treatment without buckling and kinking to a harmful degree. If the film does not have the dyed layer, but the treatment, as 45 described above, is nevertheless applied to its rear face, the curling tendency will be similarly lessened regardless of the absence of dye.

50 Where dye is to be entirely removed from colored film scrap or old colored film, the material is moved through the bath without the convolutions of the film touching each other, or it may be chopped into small 55 pieces and the latter acted upon by the mixture. Preferably, the bath is agitated in any event. The liquid, when working on a large scale, can conveniently flow counter to the movement of the film base being treated.

60 An advantage of our process in connection

with scrap is the fact that the dye is thoroughly and rapidly leached out without dissolving the film, the latter being in condition for the well known recovering processes. If the scrap were dissolved, the dye 70 would be all the more thoroughly mixed in the nitrocellulose.

Of course, many equivalent baths which include solvents or mixtures of solvents and non-solvents may be employed. Moreover, 75 if the solvents have a solvent action with respect to the fillers or softeners in the support, no harm is done. The acetone, given in the above example, has a solvent tendency 80 with respect to many of the common softeners in nitrocellulose films and yet it is successful in the above described example. Another instance of useful baths is methyl alcohol mixed with butyl alcohol or water, a convenient bath being 85 parts of methyl 85 alcohol to 15 parts of butyl alcohol by weight. It will be noted that the baths given by way of example are substantially free from mineral matter and substances of such high boiling point that they would remain on the rear face of the film in quantities sufficient to impair the latter.

Having thus described our invention, what we claim as new and desire to secure by Letters Patent is:

1. The process of treating nitrocellulose film support having a free rear face, which comprises acting on said rear face with a nitrocellulose solvent substantially free from non-volatile substances until said solvent 100 penetrates through said rear face, and stopping said action before the body of the film support is acted on.

2. The process of treating nitrocellulose film support having a rear face substantially 105 uniformly accessible to solvents, which comprises temporarily softening the material of said support at said rear face by applying to said face a volatile solvent thereof, substantially free from non-volatile ingredients, 110 stopping the action of said solvent before nitrocellulose is substantially dissolved away thereby, and evaporating applied solvent from said face.

3. The process of treating cellulose film support having dye therein adjacent the rear free face thereof, which comprises acting on said face with a liquid which has a solvent effect on said dye and sufficient solvent tendency toward said film to penetrate the latter, and limiting the action of said liquid to avoid substantial dissolving away of said cellulosic film.

4. The process of simultaneously removing dye and lessening the curling tendency 125 of nitrocellulose film support which has dye therein adjacent its free rear face, which comprises acting on said face with a liquid which has a solvent effect on said dye and sufficient solvent tendency toward said nitro-

cellulose to penetrate to the dye, and stopping the action of said liquid before it substantially dissolves away nitrocellulose from said support.

5. The process of removing dye from dyed cellulosic films impermeable to water, which includes the step of treating a face of said film with a liquid which has a solvent action on said dye and a temporary softening action on said cellulosic films without dissolving the latter during the removal of the dye, said face being all accessible to said liquid.
6. The process of removing dye from dyed cellulosic film impermeable to water which includes the step of treating said film with a liquid containing a substance which is a solvent of said film and a substance which is a non-solvent of said film, at least one of said substances being a solvent of said dye, the proportion of film solvent being sufficient to temporarily soften the film for penetration of said dye solvent without substan-

tially dissolving the film during the removal of the dye.

7. The process of removing dye from dyed cellulosic film impermeable to water, which includes the step of treating said film with a solvent of said film mixed with water, the mixture being a solvent of said dye, and the proportion of film-solvent being insufficient to dissolve the film during the removal of the dye, but sufficient to temporarily penetrate said film.

8. The process of removing dye from a dyed nitrocellulose film impermeable to water, which includes the step of treating said film with a mixture of 70 parts of acetone and 30 parts of water until the desired degree of removal is reached.

Signed at Rochester, New York, this 31st day of December, 1923.

HENRY E. VAN DERHOEF.  
JACKSON B. WELLS.

- cellulose to penetrate to the dye, and stopping the action of said liquid before it substantially dissolves away nitrocellulose from said support.
5. The process of removing dye from dyed cellulosic films impermeable to water, which includes the step of treating a face of said film with a liquid which has a solvent action on said dye and a temporary softening action 10 on said cellulosic films without dissolving the latter during the removal of the dye, said face being all accessible to said liquid.
6. The process of removing dye from dyed cellulosic film impermeable to water which 15 includes the step of treating said film with a liquid containing a substance which is a solvent of said film and a substance which is a non-solvent of said film, at least one of said substances being a solvent of said dye,
- 20 the proportion of film solvent being sufficient to temporarily soften the film for penetration of said dye solvent without substan-
- tially dissolving the film during the removal of the dye.
7. The process of removing dye from dyed cellulosic film impermeable to water, which includes the step of treating said film with a solvent of said film mixed with water, the mixture being a solvent of said dye, and the proportion of film-solvent being insufficient 25 to dissolve the film during the removal of the dye, but sufficient to temporarily penetrate said film.
8. The process of removing dye from a dyed nitrocellulose film impermeable to 30 water, which includes the step of treating said film with a mixture of 70 parts of acetone and 30 parts of water until the desired degree of removal is reached.

Signed at Rochester, New York, this 31st 40 day of December, 1923.

HENRY E. VAN DERHOEF.  
JACKSON B. WELLS.

#### Certificate of Correction.

It is hereby certified that in Letters Patent No. 1,525,761, granted February 10, 1925, upon the application of Henry E. Van Derhoef and Jackson B. Wells, of Rochester, New York, for an improvement in "Processes of Treating Cellulosic Films," an error appears in the printed specification requiring correction as follows: Page 2, line 115, claim 3, for the word "cellulose" read *cellulosic*; and that the said Letters Patent should be read with this correction therein that the same may conform to the record of the case in the Patent Office.

Signed and sealed this 31st day of March, A. D. 1925.

[SEAL.]

KARL FENNING,  
Acting Commissioner of Patents.

**Certificate of Correction.**

It is hereby certified that in Letters Patent No. 1,525,761, granted February 10, 1925, upon the application of Henry E. Van Derhoef and Jackson B. Wells, of Rochester, New York, for an improvement in "Processes of Treating Cellulosic Films," an error appears in the printed specification requiring correction as follows: Page 2, line 115, claim 3, for the word "cellulose" read *cellulosic*; and that the said Letters Patent should be read with this correction therein that the same may conform to the record of the case in the Patent Office.

Signed and sealed this 31st day of March, A. D. 1925.

[SEAL.]

KARL FENNING,  
*Acting Commissioner of Patents.*